

## United States Patent Office

2,727,804

Patented Dec. 20, 1955

1

2,727,804

## BLEACHING OF POLYAMIDES

Albertus Gerardus Lutgerhorst, Arnhem, Netherlands, assignor to N. V. Onderzoekingsinstituut Research, Arnhem, Netherlands, a corporation of the Netherlands

No Drawing. Application April 9, 1953,  
Serial No. 347,839

Claims priority, application Netherlands August 7, 1952

7 Claims. (Cl. 8—109)

This invention relates to the bleaching of textile materials made of synthetic linear polyamides of the nylon type. Examples of such synthetic linear polyamides are those described in U. S. patents such as Nos. 2,071,250, 2,071,253, 2,130,948 and 2,359,877. These synthetic linear polyamides are characterized by the presence of repeating carbonamide units having the structural formula



One of the principal objects of the present invention is to provide a new and improved method for bleaching textile materials of the kind indicated, either in the form of artificial threads or fibers or in the form of fabrics knit or woven from such threads or fibers, in such manner as to bleach them without impairing the strength of the fibers in any way. A further object of the invention is to provide a method for successfully bleaching polyamide materials of the foregoing nature with hypochlorite solutions while avoiding previously known disadvantages attendant upon the use of hypochlorite solutions for the purpose indicated.

The manner in which these and other objects and features of the invention are attained will appear more fully from the following description thereof, in which reference is made to typical and preferred procedures in order to indicate more fully the nature of the invention but without intending to limit the invention thereby.

It has long been known in the art that the bleaching of textile materials consisting essentially of synthetic linear polyamides gives rise to serious difficulties. This is true both for fibers and threads consisting of these polyamides as well as for fabrics knit or woven from such fibers or threads, and especially in the case of finished articles made from such knit or woven fabrics. One of the more serious difficulties known to be encountered in the case of treatment of these materials is that upon high temperature stabilization, known per se, a slight discoloration often results.

It is also known that if one attempts to bleach these synthetic linear polyamide materials with hypochlorite solutions, such as NaOCl or Ca(OCl)<sub>2</sub> solutions, a considerable amount of chlorine is adsorbed or chemically bound by the fiber or thread undergoing treatment, which chlorine is not removed by any normal treatment with known anti-chlor agents. Owing to this retained residual chlorine, there occurs a serious decline in the strength of the fibers making up the textile material so that as a consequence the bleaching of nylon fabrics with hypochlorite solutions cannot be employed, and the literature warns against it. Even treatment with anti-chlor reagents at somewhat increased temperatures, e. g., 40–60° C., has been found to give no improvement in this respect, and consequently such fabrics have heretofore been of necessity bleached with chlorite solutions, such as NaClO<sub>2</sub>, in acid medium. Although good results may be obtained in this way, nevertheless the step of bleaching with chlorite entails considerable technical objections because the chlo-

2

rite—especially in the somewhat acid solutions and at the relatively high temperatures employed required for its use in bleaching—is extremely reactive with respect to almost all materials of construction that would normally be employed for constructing the apparatus in which the bleaching treatment is carried out. Moreover, the ClO<sub>2</sub> that may be evolved from the chlorite solution is extremely toxic.

In accordance with the present invention, however, it has been discovered that all textile materials consisting essentially of synthetic linear polyamides may be bleached with excellent results without impairing the strength of the fiber provided said textile materials are first treated with a hypochlorite solution and then with a reducing agent at a temperature above 80° C.

Particularly desirable results are obtained when one employs as the reducing agent a solution of a hydrosulfite (Na<sub>2</sub>S<sub>2</sub>O<sub>4</sub>) or one of its derivatives at a temperature of 90–95° C.

10 The antecedent bleaching operation may be performed in different ways and also at widely differing pH values. For example, the bleaching may be performed at room temperature with a hypochlorite solution containing 0.5 g./l. of active chlorine at a pH of either 8–10 or 3–4, and over a period that may vary from 15 minutes to 2 hours. Thereupon, an aftertreatment with a hydrosulfite solution (for example, 1 g./l. of Na<sub>2</sub>S<sub>2</sub>O<sub>4</sub>) at 90–95° C. completely removes all the retained chlorine from the fiber. For this purpose a time of treatment of five minutes is generally sufficient, but this may be extended for example to 30 minutes, if desired.

15 Although nearly all the ordinary reducing agents such as aqueous solutions of bisulfite, thiosulfate, sulfite, and similar reagents have been found to be capable of removing the retained chlorine from the nylon articles during the subsequent anti-chlor treatment at temperatures higher than 80° C., the bleaching effect obtained was sometimes less satisfactory than after a treatment with aqueous solutions of hydrosulfite and its derivatives, such as the formaldehyde addition compound or the zinc-formaldehyde addition compound of hydrosulfite. These latter compounds have the additional advantage of being more stable at the relatively high temperatures employed for the aftertreatment, and are therefore preferred.

20 The outstanding effect obtained in accordance with the method of the present invention is all the more surprising, since the application to the nylon fabric of a reducing agent alone, even at high temperature, results in only a very slight bleaching effect.

25 The presence or absence of retained chlorine can easily be shown by means of an acidified potassium iodide solution which, even in the presence of mere traces of chlorine in the material, gives an intensive yellow coloration. As soon as all the residual chlorine has been removed, however, no coloration occurs upon testing with the acidified potassium iodide solution.

30 After rinsing and drying the nylon articles bleached according to the method of the present invention, the whiteness thereof is as good as, or frequently even better than, that which can be obtained by bleaching with a chlorite solution. It will be apparent therefore that when proceeding in accordance with the present invention all the objections inherent in carrying out the bleaching operation with chlorite (ClO<sub>2</sub>) are eliminated, and at the same time the conventional apparatus known in the art for bleaching with hypochlorite may be employed.

35 The bleaching agent may be employed in the form of calcium hypochlorite solutions or alkali metal hypochlorite solutions such as sodium or potassium hypochlorite solutions, and the reducing agents may be employed in the form of their alkali metal salt solutions such as sodium or potassium salt solutions or, in the case of the hydrosul-

fite, solutions of the addition compounds referred to above.

I am aware that it has been suggested heretofore to bleach nylon fibers and the like with sodium hypochlorite solution followed by decoloration in an acid sodium bisulfite bath (see Diserens, *Neueste Fortschritte und Verfahren in der chemischen Technologie der Textilfasern*, Part 2, *Neue Verfahren in der Technik der chemischen Veredlung der Textilfasern*, vol. I, paragraph bridging pages 577-8) but there is no indication in Diserens that the subsequent antichlor treatment must be conducted at relatively high temperatures. In fact, Diserens indicates that while in many cases his process gives good results, nevertheless it is insufficient for pure white and he goes on to recommend bleaching with sodium chlorite or with chlorine dioxide.

While specific examples of preferred methods and reagents embodying the present invention have been described above, it will be apparent that many changes and modifications may be made in the methods of procedure and in the reagents without departing from the spirit of the invention. It will therefore be understood that the examples recited and the particular proportions and methods of procedure set forth above are intended to be illustrative only, and are not intended to limit the invention.

What is claimed is:

1. A method for the bleaching of textile materials comprising a synthetic linear polyamide comprising treating such materials with a hypochlorite, and then with a reducing agent at a temperature above 80° C.

2. A method for the bleaching of textile materials comprising a synthetic linear polyamide comprising treating such materials with a solution yielding hypochlorite ions, and then with a solution of a reducing agent at a temperature higher than 80° C.

3. A method for the bleaching of textile materials comprising a synthetic linear polyamide comprising bleaching such materials with an aqueous solution of a hypochlorite selected from the class consisting of calcium and alkali metal hypochlorites, and then with an aqueous solution of a reducing agent at a temperature of about 90-95° C.

4. A method as defined in claim 3 wherein the reducing agent is a hydrosulfite.

5. A method for the bleaching of textile materials comprising a synthetic linear polyamide comprising treating

such materials with an aqueous solution yielding hypochlorite ions, rinsing the textile materials in order to remove most of the hypochlorite solution, and thereafter removing residual chlorine from said textile materials by treating same with an aqueous solution of a compound selected from the class consisting of hydrosulfites and addition compounds of hydrosulfites at a temperature above 80° C.

above 35 °C.

6. A method for the bleaching of textile materials comprising a synthetic linear polyamide comprising treating such materials with an aqueous solution of a hypochlorite selected from the class consisting of calcium and alkali metal hypochlorites, rinsing the textile materials in order to remove most of the hypochlorite solution, and thereafter removing residual chlorine from said textile materials by treating same with an aqueous solution of a compound selected from the class consisting of hydrosulfites and addition compounds of hydrosulfites at a temperature of approximately 90-95 °C.

20 7. A method for the bleaching of textile materials comprising a synthetic linear polyamide comprising treating such materials with an aqueous solution of a hypochlorite selected from the class consisting of calcium and alkali metal hypochlorites, rinsing the textile materials in order  
25 to remove most of the hypochlorite solution, and thereafter removing residual chlorine from said textile materials by treating same with an aqueous solution of sodium hydrosulfite at a temperature of approximately 90-95° C.

**References Cited in the file of this patent**

UNITED STATES PATENTS

2,260,367 Dubeau ----- Oct. 28, 1941

## FOREIGN PATENTS

35 682,975 Great Britain ----- Nov. 17, 1952

#### OTHER REFERENCES

Turnbull: "Dyeing of Broad-Woven Nylon Fabrics," Am. Dyest. Reporter, October 17, 1949, p. 747.

40 Diserens: "Neueste Fortschritte und Verfahren in der chemischen Technologie der Textilfasern," part 2, Neue Verfahren in der Technik der chemischen Veredlung der Textilfasern, vol. 1, pp. 577 to 580, Birkhauser, Basel, 1948.

45